

2,975,112

## ELECTRODEPOSITION OF ZINC

Edward B. Saubestre, Elmhurst, N.Y., assignor, by mesne assignments, to Sylvania Electric Products Inc., Wilmington, Del., a corporation of Delaware

No Drawing. Filed Jan. 4, 1955, Ser. No. 479,842

4 Claims. (Cl. 204—119)

This invention relates to the electrodeposition of zinc, and more particularly to the electrowinning of zinc from zinc solutions containing germanium as an impurity.

Germanium is a metal which at present is in great demand because of its extremely valuable properties in electrical and electronic circuits. Accordingly, ores containing this metal are being currently processed in great quantities. Such ores usually contain relatively large amounts of zinc, whereby zinc sulfate residues in solution form are obtained. Similar solutions are obtained as an intermediate step in the extraction of other metals, including zinc itself, from ores or other materials with sulfuric acid.

The art of recovering zinc from acid solutions of zinc sulfate by electrolytic means is of course old and well known. However, in attempting to extract zinc by such means from zinc sulfate solutions (obtained as a residue from the manufacture of germanium), difficulty was encountered. Little or no plating of zinc on the cathode could be achieved. This difficulty was traced to the presence of small quantities of germanium present in the zinc sulfate solution, despite all the previous steps taken to extract the germanium. Amounts of germanium as low as 1 mg./l. were found to be sufficient to prevent deposition of zinc.

While the presence of certain impurities in electrolytes is known often to cause great difficulty during the operation of plating by electrolytic methods, most if not all of the expedients heretofore employed for solving this problem have been directed towards a preliminary treatment of the electrolyte to remove the undesired impurities. As examples of some of these proposed preliminary purification methods, reference may be had to U.S. Patents Nos. 2,396,569, 2,405,302, 2,503,479, 2,509,916, 2,509,917, and 2,509,918. Although these methods have been generally found to be ineffective for removing germanium from the zinc electrolyte solutions being dealt with, one such pre-purification method has been found satisfactorily employed to remove the germanium. It involves absorbing and removing the germanium from solution by means of ferric hydrate precipitated by zinc oxide in the leaching operation.

The aforementioned pre-purification method for removing the undesirable germanium has, however, several disadvantages. In common with other pre-purification methods, it involves additional equipment and steps, including a filtration which is not easily effected. Further, it requires the deliberate addition of iron to ores which may have a relatively high germanium content and a low iron content which also introduces another element to control with the attendant problem of human error in actual plant operation.

It is accordingly an object of this invention to provide a method for the electrodeposition of zinc which avoids one or more of the above-described difficulties and disadvantages. A further object of this invention is to provide a method for the electrodeposition of zinc from a zinc electrolyte solution containing germanium as an

impurity. Other objects and advantages will appear as the description proceeds.

The attainment of the above objects is made possible by the instant invention which comprises maintaining the pH of the electrolyte within a range of about 3.0 to 3.5 during electrowinning. While this may be accomplished in any convenient way, it has been found that best results may be obtained by adding a strong inorganic base to the electrolyte in such manner as to maintain the pH within a range of about 3.0 to 3.5 during the electrolysis. This method has been found to enable satisfactory plating of zinc over extended periods of time despite the presence of up to about 0.01 g./l., or more of germanium oxide in the electrolyte. When the pH is allowed to go below about 3.0, the cathode efficiency begins to drop rapidly, while at a pH of about 4 or more, a heavy precipitate forms with consequent drop in efficiency.

The improved results attained by the instant process are surprising in view of the many advantages attributable to operation at high acid concentration (low pH). Thus, a high acid concentration increases the conductivity of the electrolyte, which enables the use of a higher current density or a lower voltage at the same current density. High current densities are of course economically desirable. In addition, high acid concentration inhibits sponging caused by precipitation of oxides or basic salts or other impurities. Accordingly, most expedients heretofore employed for controlling pH have involved use of acids of various types, acid salts, soluble anodes, diaphragms, and the like. As a matter of fact, some electrolytic processes deliberately operate at an extremely low pH depending upon the continuous formation of free acid known to occur when using insoluble anodes, for use in a recycling process to dissolve further quantities of zinc from ores containing same.

In carrying out a preferred embodiment of the process of the instant invention, a strong inorganic base such as lithium hydroxide but more preferably sodium or potassium hydroxide, is added periodically or continuously as needed to maintain the pH of the bath within the required range. Although the base may be added as a solid, it is preferably added in the form of a concentrated aqueous solution to promote more rapid neutralization and pH control without unduly diluting the bath. For most practical purposes, concentrations of about 15 to 50% by weight are operative, a range of about 20 to 40% being preferred.

The pH of the bath should be periodically or continuously measured, and this may be carried out in any manner well known in the art. Since insoluble anodes are employed, the tendency of the pH is to fall below the minimum value of about 3.0 as required herein, and chemical colorimetric indicators or test papers may be employed to determine when the pH approaches or falls below this value. As such indicators, there may be mentioned Butter Yellow, Congo Red, 2,5-dinitrohydroquinone, Bromophenol Blue, Methyl Orange and the like. Change of color of the indicator as the pH of the electrolyte solution falls below 3.0 shows the need for addition of the base, which may be accomplished manually or by automatically controlled means. When working with a particular type of electrolyte solution from a given source the worker skilled in the art will readily ascertain, after one or more runs, the approximate rate of addition of the base necessary to maintain the pH within the required range. The required addition may then be made manually at periodical intervals, or either periodically or continuously by automatic means, and the pH measured only occasionally as a check.

Automatic control is of course highly desirable and should be made use of where possible. Merely by way

of illustration, means may be installed for automatically extracting a test portion of the electrolyte solution, and measuring its pH by proper instrumentation. Means responsive to the measured pH may then be provided for automatically adding the base to the electrolyte solution in predetermined increments sufficient to prevent the pH from falling below the minimum value of about 3.0.

The electrolytic process is otherwise carried out in a well known manner. Insoluble anodes are employed, such as lead, lead-silver, silicon-iron, lead-thallium-calcium, lead peroxide, manganese dioxide, or the like. Choice of material for the cathode will of course depend upon the object in view, which may be to recover zinc in substantially pure form, to plate articles with zinc, or the like. In the latter case, the article to be coated, which may be iron or steel, aluminum, zinc or the like, is employed as the cathode. In the former case, the cathode should be of such nature as to permit the zinc to be readily detached therefrom, as for example, oiled or graphite-covered copper or aluminum. Alternately, the cathode may be electrolytic zinc foil, whereby it may be melted down as a unit. Another expedient which may be employed involves the use of iron or other high melting point material as the cathode followed by removal of the zinc deposited thereon by dipping the cathode in a bath of molten zinc, fused zinc chloride or the like. Current densities of the order of about 50 to 600 amperes per square foot may be used with good results. The zinc content of the bath is replenished from time to time by addition of more zinc sulfate solution which may contain germanium as an impurity as above-mentioned. The pH of the replenishing zinc sulfate solution may vary from the range required in the instant invention provided of course it is not added in such a manner as to carry the pH of the electrolytic bath outside said range.

The following example is illustrative of a preferred embodiment of this invention and is not to be regarded as limitative:

*Example*

A zinc sulfate solution, obtained as a residue from the manufacture of germanium at Towanda, Pa., was examined and found to have a pH of 4.0 to 4.5 and to contain 100 g./l. of zinc and .006 g./l. of  $\text{GeO}_2$ . This solution was employed as the electrolyte bath for the electrodeposition of zinc using platinum anode and 1010 cold rolled steel cathode at a current density of 80 amperes per square foot, and at a pH maintained within the range of 3.1 to 3.3 (colorimetric) by measurement with indicator paper (2.7-4.7) made by Anachemia, Ltd. and periodic addition of a 24% by weight aqueous solution of sodium hydroxide. The process was run for several days, with replenishment of metal content from time to time by addition of further amounts of the original zinc sulfate solution. Good quality plates of zinc in thicknesses of up to 1.5 mils were obtained, at cathode efficiencies of 80% to 90%, with substantially no loss in

efficiency or change in appearance of plate throughout the run.

This invention has been disclosed with respect to certain preferred embodiments, and various modifications and variations thereof will become obvious to the person skilled in the art. It is to be understood that such modifications and variations are to be included within the spirit and purview of this application and the scope of the appended claims.

What I claim is:

1. A method of extracting zinc from baths containing zinc salts and germanium as an impurity including the steps of making said bath containing zinc salts and germanium the electrolyte in the presence of an insoluble anode and a cathode, raising the pH of said bath to within the range of 3.0 to 3.5 and thereafter maintaining the pH within said range, and electrowinning zinc at said cathode despite the germanium content of said bath.

2. A method of extracting zinc from baths containing zinc salts and germanium as an impurity including the steps of making said bath containing zinc salts and germanium the electrolyte in the presence of an insoluble anode and a cathode, raising the pH of said bath to within the range of 3.0 to 3.5 by the addition of a strong inorganic base and thereafter maintaining the pH within said range, and electrowinning zinc at said cathode despite the germanium content of said bath.

3. A method of extracting zinc from baths containing zinc salts and germanium as an impurity including the steps of making said bath containing zinc salts and germanium the electrolyte in the presence of an insoluble anode and a cathode, raising the pH of said bath to within the range of 3.0 to 3.5 by the addition of alkali-metal hydroxide selected from the group consisting of sodium and potassium hydroxide and thereafter maintaining the pH within said range, and electrowinning zinc at said cathode despite the germanium content of said bath.

4. A method of extracting zinc from baths containing zinc salts and germanium as an impurity including the steps of making said bath containing zinc salts and germanium the electrolyte in the presence of an insoluble anode and a cathode, raising the pH of said bath to within the range of 3.0 to 3.5 by the addition of a concentrated aqueous solution containing an alkali-metal hydroxide and thereafter maintaining the pH within said range, and electrowinning zinc at said cathode despite the germanium content of said bath.

References Cited in the file of this patent

UNITED STATES PATENTS

2,576,998 Main et al. ----- Dec. 4, 1951

FOREIGN PATENTS

693,606 Great Britain ----- July 1, 1953